

## UNITED STATES PATENT OFFICE

2,281,598

## SOLVENT AND FUEL CONTAINING SAME

Carl F. Prutton, Cleveland Heights, Ohio, assignor, by direct and mesne assignments, to The Lubri-Zol Corporation, Wickliffe, Ohio, a corporation of Ohio

No Drawing. Application March 17, 1939,  
Serial No. 262,504

6 Claims. (Cl. 44—9)

This invention relates, as indicated, to a new solvent, and also to such fuel as is consumed by internal combustion engines which has added thereto my new solvent in order to increase the efficiency of operation of the engine. This application is in part a continuation of applicant's co-pending application Serial No. 107,228, filed October 23, 1936. This application is also a continuation-in-part of my copending application, Serial No. 737,070, filed July 26, 1934.

It is a fact, generally known, that so-called "carbon" deposits form on the cylinder walls, pistons, valves, etc., making for inefficient operation of the engine due to such consequences as:

1. Carbon on piston head and cylinder head increases the knock susceptibility of a motor.

2. Carbon on piston head and cylinder head causes higher temperatures to be maintained, sometimes resulting in pre-ignition.

3. Carbon around the spark plug frequently causes shorting of the plug, which means that the cylinder will not fire.

4. Carbon around and behind piston rings causes the rings to "set," lowering compression, increasing oil consumption and decreasing power.

5. Carbon around valve seats and valve stems will not allow the valves to close properly, which causes decreased compression, burning of the valves, loss of power, etc.

The formation of these deposits, which consist of carbon and other solids bound together by gummy binders, occurs whenever any of the ordinary fuels is used and necessitates more frequent engine overhauls than would otherwise be required, such overhauls being a source of continual annoyance and expense.

Midgley, in Patent No. 1,668,022 has disclosed the use of tetra-ethyl lead and a volatile bromide compound in an internal combustion engine fuel for the purpose of suppressing engine-knock, the bromide compound in certain respects inhibiting the deleterious effects of lead deposits, and such a mixture is now commonly employed. However, the combustion of the fuel thus improved gives rise to other problems, the solution of which is among the objects of this invention.

It has been discovered that these "carbon" deposits resulting from the combustion of internal combustion engine fuels contain a binder which has two principal components: (1) condensed and/or polymerized hydrocarbons and (2) more or less oxidized condensed and/or polymerized hydrocarbons. I have found that the best solvents for component (1) are not the best solvents for component (2) and that the best solvent for the binder is a combination of the two types of solvents respectively best suited to dissolve the

separate components of the binder. For addition to the fuel, it is obvious that solvents must be found which are mutually compatible, soluble or miscible in the fuel, or capable of forming a stable form of suspension or emulsion and which will dissolve the two sorts of gummy binders previously referred to.

It is, therefore, among the objects of my invention to provide a new solvent which will be effective in the removal of carbon deposits of the sort found in internal combustion engines by acting upon the gummy binders in the deposit composition.

It is also among the objects of this invention to provide an engine fuel suitable for consumption by internal combustion engines, and which has mixed therewith my improved solvent which will inhibit the formation of these carbon deposits and aid in the removal of any already formed.

Another object of this invention is to provide an engine fuel having all of the above-named desirable characteristics and which, in addition, has the further effect of aiding in the carrying off of the metal when such compounds as lead tetra-ethyl are utilized in the fuel, this composition being non-corrosive in use.

Other objects of the invention will appear as the description proceeds.

To the accomplishment of the foregoing and related ends, said invention then consists of the means hereinafter fully described and particularly pointed out in the claims.

The following description sets forth in detail certain approved combinations of ingredients embodying my invention, such disclosed means constituting, however, but certain of various forms in which the principle of the invention may be used.

Broadly stated, this invention comprises a new solvent for condensed and/or polymerized organic materials and especially for such materials containing a combination of condensed and/or polymerized hydrocarbons and condensed and/or polymerized oxidized hydrocarbons, said solvent containing a mixture of at least one each of certain halogenated oxygen-free organic compounds and at least one each of certain oxygen-bearing organic compounds. Of these latter compounds some are more effective in some services if halogenated and more effective in other services and under different conditions is unhalogenated.

An important use for my new solvent is in dissolving the binder of carbon deposits usually found in the combustion chambers of internal combustion engines. For this reason the succeeding paragraphs are largely a description of

such use and especially of engine fuels designed to have this and other desirable effects. My new solvent may, however, be utilized whenever deposits of the general type described are encountered.

As is hereinafter more particularly pointed out, the above defined components of the solvent comprising this invention will preferably and for best results have certain physical and chemical characteristics which especially adapt such components and the solvent containing the same for use in conjunction with the principal types of engine fuel in common use today.

The components of the solvent should be of low volatility, i. e., with a vapor pressure at a 15 temperature of 170° C. of below atmospheric and capable of boiling at atmospheric pressure without substantial decomposition. In one embodiment of my invention now in commercial use, one component of my new solvent has a vapor pressure less than atmospheric at a temperature above 300° C. A mixture of two components, one with a vapor pressure a little below atmospheric at 170° C. and the other with a vapor pressure a little below atmospheric at 350° C., has 25 proven highly satisfactory.

#### Oxygen free component

I have found that the halogenated oxygen-free 30 organic compounds usable as a component in my new solvent, as above defined, should be of the type which are substantially stable under the rather severe conditions encountered in the combustion chamber of internal combustion engines. 35

Of the aromatic compounds which are thus available, those which are of the "non-condensed" ring type will be found sufficiently stable for the purposes above defined. Poly-nuclear aromatic compounds (that is, those containing 40 more than one ring) of the "non-condensed" ring type are thus the more desirable of the stable aromatic compounds which are available for use.

As hereinafter pointed out, certain of the aliphatic compounds are likewise suitable although, in general, the aliphatic compounds will be found to be less stable than the type of aromatic compounds above referred to which is suitable for use.

In the case of the halogenated aromatic oxygen-free compounds, it is preferable that the halogen be attached to a carbon atom of the 50 benzenoid ring. These latter compounds are usually more desirable because of their non-corrosive character and general stability.

The halogenated oxygen-free organic compounds as noted may be either:

#### A. Aliphatic, such as halogenated:

##### I. Hydrocarbons,

Notably, those containing from four to ten carbon atoms, e. g.: 60  
 Fluorinated hexane  
 Fluorinated octane  
 Fluorinated decane

##### II. Amines

Primary, secondary and tertiary, 65  
 e. g., hexylamines, di-amylamines, tri-amylamines, such as:  
 Fluorinated tri-amyl amine  
 Fluorinated hexyl amines  
 also:

Fluorinated tributyl amine

##### III. Nitriles

Halogenated ethyl nitrile  
 Halogenated butyl nitrile

or the more generally preferable:

#### B. Cyclic compounds, such as halogenated:

##### I. Benzene and related compounds such as:

(1) Halogenated benzene, e. g.:  
 The dichlorbenzenes, notably the ortho compound

The ortho-dibrom benzenes  
 The fluorinated benzenes

(2) Halogenated derivatives of benzene such as:

(a) Halogenated homologs of benzene, e. g.:

Mono-chlor xylene  
 Mono-chlor cymene  
 Ethyl mono-chlor benzenes  
 Propyl mono-chlor benzenes  
 Di-ethyl mono-chlor benzenes

Ethyl dichlor benzenes  
 Propyl dichlor benzenes  
 Di-ethyl dichlor benzenes

(b) Halogenated amino derivatives of benzene, e. g.:

Chlorinated aniline  
 Mono-chlor aniline (preferably the ortho-compound)  
 Mono-chlor di-methyl aniline

Chlorinated toluidines  
 Chlorinated xylidines  
 Chlorinated diphenylamine

(c) Halogenated hydrobenzenes, e. g.:

Hydrogenated dichlor-benzenes  
 Dichlorhexahydrobenzene  
 (Dichlor cyclohexane)

(3) Aromatic nitriles, e. g., chlorinated phenyl nitrile

#### II. Polyphenyls, and related compounds, including diphenyl, diphenyl benzenes, etc., such as,

(1) Chlorinated diphenyl, e. g.:

Mono-chlor diphenyls  
 Di-chlor diphenyls  
 Tri-chlor diphenyls

(2) Brominated diphenyl, e. g., the mono-brom diphenyls

(3) Fluorinated diphenyl

(4) Halogenated derivatives of diphenyl, such as,

(a) Halogenated homologs of diphenyl, e. g.:

Chlorinated methyl diphenyls  
 Chlorinated ethyl diphenyls

(b) Halogenated amino derivatives of diphenyl, e. g.:

Chlorinated amino-di-phenyls  
 Chlorinated amino methyl diphenyls

(c) Halogenated hydrodiphenyls, e. g.:

Chlorinated phenyl hexahydrobenzene  
 Chlorinated dodecahydrodiphenyl

#### IV. Bridged ring compounds, such as the terpenes and related compounds, and their derivatives, e. g., chlorinated pinene.

#### V. Heterocyclic compounds, such as pyridine, quinoline, pyrrole, thiophene, and derivatives of them, e. g., mono-chlor pyridine.

Very satisfactory results may be obtained when two or more different halogens are present in the same molecule, orthobrom-chlor benzene, ethyl-orthobrom chlor benzene, and the fluorinated chlorine compounds being good examples of such compounds. If the aromatic compounds have been alkylated they are often especially effective.

As a matter of convenience, the halogenated diphenyls and substituted diphenyls, as well as halogenated substituted benzenes where two or more phenyl groups are directly linked, may be inclusively referred to as halogenated polyphenyls.

Some of the best examples of the aromatic solvents are:

Chlorinated benzene, B-I. (1), e. g.: 15

Di-chlor benzene (notably the ortho compound)

Chlorinated ethyl benzene

Chlorinated diphenyl B-II. (1)

Chlorinated aniline B-I. (2) (b)

Chlorinated pyridine B-VIII.

Chlorinated quinoline B-VII.

Good examples of halogenated aliphatic hydrocarbons are:

Fluorinated pentane 25

Fluorinated hexane

Fluorinated octane

Halogenated petroleum derivatives, particularly halogenated petroleum oils and waxes. 30

*Oxygen-bearing component*

I have found that of the entire class of oxygen bearing organic compounds usable as a component of my new solvent, as above defined, 35 the halogenated compounds and preferably those of the aromatic series are generally superior solvents for the oxidized polymerized hydrocarbon deposit, and that these solvents may be used in conjunction with the solvents for the unoxidized 40 condensed and/or polymerized hydrocarbon deposit, also being compatible with the fuel. Here again, compounds of the aromatic series with the halogen attached to the ring are favored. However, a certain number of the oxygen-bearing aliphatic compounds have been 45 found to be very effective.

The oxygen-bearing components may, for convenience, be classified as follows:

I. Aliphatic, or carbon chain type 60

Oxygen-bearing derivatives of:

- A. Hydrocarbons of the paraffin series,
- B. Hydrocarbons of the olefine series and
- C. Hydrocarbons of the acetylene series, 55

II. Organic ring type

Oxygen-bearing derivatives of:

A. "Carbon ring" type compounds

- (a) Of the aromatic, or allied type, including oxygen-bearing derivatives of benzene, naphthalene, anthracene, etc., also compounds of the bridged ring type, such as the terpenes, and related compounds.

- (b) Of the class including the cyclo-paraffins, cyclo-olefines, etc. Examples of this class are oxygen-bearing derivatives of the following:

- (1) Hydrogenation products of benzene (e. g. cyclohexane, cyclo-hexene, cyclohexadiene); such as hydrogenated phenol, notably: cyclohexanol, di-hydro-phenol, tetra-hydro-phenol. 70

75

- (2) Hydrogenation products of naphthalene (e. g. decahydro-naphthalene, tetrahydro-naphthalene, etc.); such as the hydrogenated naphthols.
- (3) Naphthenes, such as naphthenic acid, etc.
- (c) Of mixed type such as derivatives of indene, hydrindene, hydranthracene, etc.

#### B. Heterocyclic type compounds

- (a) Of the aromatic or allied type including derivatives of pyridine, quinoline, etc.
- (b) Other types such as furfural, furan and its derivatives and derivatives of thiophene, pyrrole, etc.

The oxygen-bearing derivatives of the foregoing compounds may also be classified according to the nature of the attachment of the oxygen to the molecule, viz:

I'. Directly attached to one or more carbon atoms, as in the case of:

- (1') Ethers and analogous compounds
- (2') Compounds containing the



radicle, such as alcohols and other derivatives of carbinol (including phenols, cresols, naphthols etc.)

- (3') Compounds containing the carbonyl



radicle, such as amides, aldehydes, ketones, organic acids, esters and salts of organic acids, thio-acids and esters of thio-acids

- (4') Compounds in which oxygen forms a part of the ring structure, e. g. furan and its derivatives, etc.
- (5') Compounds with inorganic radicle where the oxygen is directly attached to carbon atom

Arsenite  
Hypochlorite  
Phosphite  
Thiophosphate  
Thiophosphite  
 $\beta$ -Hydroxylamines

II'. Indirectly attached through the means of some other atom, i. e., in the form of an inorganic radicle, e. g.:

Arsenate  
Chlorate  
Chlorite  
Cyanate  
 $\alpha$ -Hydroxylamine  
Nitrate  
Nitrite  
Nitro  
Nitroso  
Oxime  
Perchlorate  
Phosphate  
Sulphate  
Sulphite  
Sulphinic acid  
Sulphone  
Sulphonic acid  
Sulphoxide  
Thio-sulphate

The following table indicates some of the compounds which are especially suitable, halogenated or unhalogenated, as the case may be:

eight atoms of halogen per molecule. Chlorinated diphenyl ether which contains about six atoms of chlorine per molecule, and has prefer-

### Organic oxygen compounds

| Ring compounds                                              | Unhalogenated                                                                                                                                                                                           | Halogenated                                                                                                                                                                                                 |
|-------------------------------------------------------------|---------------------------------------------------------------------------------------------------------------------------------------------------------------------------------------------------------|-------------------------------------------------------------------------------------------------------------------------------------------------------------------------------------------------------------|
| <b>Aromatic</b>                                             |                                                                                                                                                                                                         |                                                                                                                                                                                                             |
| <b>Phenols</b>                                              | Phenol<br>α-Naphthol<br>Amino phenols<br>Butyl phenol<br>Phenyl phenol<br>Xylenol<br>"Tar acids" (preferably refined by distillation)                                                                   | O-chlor phenol<br>Monochlor α-naphthol                                                                                                                                                                      |
| <b>Alcohols</b>                                             | Benzyl alcohol<br>Phenyl ethyl alcohol                                                                                                                                                                  | Chlorbenzyl alcohols                                                                                                                                                                                        |
| <b>Aldehydes (less desirable because of polymerization)</b> | Benzaldehyde                                                                                                                                                                                            |                                                                                                                                                                                                             |
| <b>Ketones</b>                                              | Benzophenone<br>Phenyl tolyl ketones<br>Dinaphthyl ketone                                                                                                                                               | Mono-chlor benzophenone                                                                                                                                                                                     |
| <b>Amides and substituted amides</b>                        | Benzamide<br>Acetanilide<br>Stearanilide                                                                                                                                                                |                                                                                                                                                                                                             |
| <b>Acids</b>                                                | Phenyl fatty acids e. g. phenyl acetic acid                                                                                                                                                             | Chlorphenyl acetic acid<br>Chlor-salicylic acid                                                                                                                                                             |
| <b>Esters</b>                                               | Phenyl acetate<br>Phenyl carbonate<br>Ethyl benzoate<br>Butyl benzoate<br>Diethyl phthalate<br>Diethyl phthalate<br>Ethyl and butyl esters of phenyl acetic acid<br>Methyl salicylate<br>Benzyl acetate | Ethyl chlorbenzoates<br>Butyl chlorbenzoates<br>Diethyl chlorphthalates<br>Diethyl chlorphthalates<br>Ethyl and butyl esters of chlorphenyl acetic acid<br>Methyl chlor salicylates<br>Chlorbenzyl acetates |
| <b>Salts</b>                                                | Pyridine acetate<br>Quinoline acetate<br>Aniline stearate                                                                                                                                               |                                                                                                                                                                                                             |
| <b>Ethers</b>                                               | Diphenyl ether<br>Phenyl ethyl ether<br>Dixenyl ether<br>Dinaphthyl ether<br>Alkylated diphenyl ether                                                                                                   | Chlorinated diphenyl ether<br>Chlorphenyl ethyl ethers<br>Chlorinated dixenyl ether<br>Chlorinated dinaphthyl ether<br>Alkylated chlor-diphenyl ether                                                       |
| <b>Non-aromatic oxygen-bearing organic ring compounds</b>   | Naphthenic acids<br>Esters of naphthenic acids                                                                                                                                                          | Chlorinated cyclohexanol                                                                                                                                                                                    |
| <b>Oxygen-bearing heterocyclic compounds</b>                |                                                                                                                                                                                                         |                                                                                                                                                                                                             |

(1) Furane and derivatives, e. g.

Esters of pyromuic acid (furoates),

Furfuryl alcohol and esters of it, e. g. furfuryl acetate,

(2) Oxygen bearing derivatives of thiophene and pyrrole, e. g., esters of thiophene carboxylic acids and esters of pyrrole carboxylic acids.

| Chain compounds       | Unhalogenated                                                     | Halogenated                                                                                                       |
|-----------------------|-------------------------------------------------------------------|-------------------------------------------------------------------------------------------------------------------|
| <b>Alcohols</b>       | Octyl alcohol<br>Decyl alcohol<br>Lauryl alcohol<br>Cetyl alcohol | Fluorinated octyl alcohol<br>Fluorinated decyl alcohol<br>Fluorinated lauryl alcohol<br>Fluorinated cetyl alcohol |
| <b>Esters</b>         | Methyl stearate<br>Lauryl acetate                                 | Methyl dichlor stearate                                                                                           |
| <b>Hydroxy-amines</b> | Tri-ethanol amine<br>Tri-butanol amine                            |                                                                                                                   |
| <b>Ethers</b>         | Amyl ether<br>Octyl ether                                         |                                                                                                                   |
| <b>Ketone</b>         | Diethyl ketone<br>Di-ethyl ketone<br>Di-octyl ketone              |                                                                                                                   |
| <b>Acids</b>          | Lauric acid                                                       |                                                                                                                   |

A good example of a solvent of the oxygen-bearing class is chlorinated diphenyl ether, containing an average of from about three to about

55 ably been purified by vacuum distillation, or other means, is one of the most desirable solvents of this class. This solvent boils at a temperature above 300° C. without appreciable decomposition. (See my co-pending application No. 83,976.)

60 Of the above enumerated classes of oxygen-bearing compounds, the aromatic compounds are generally preferred and particularly the aromatic ethers and ketones. Another preferred class of compounds is that in which oxygen forms a part of a ring structure.

65 Since, in general, aromatic compounds containing multiple ring structures of the condensed type such as naphthalene, anthracene, phenanthrene, etc. (that is, of the type in which certain carbon atoms are contained in or common to two rings) are more easily oxidized, and, therefore, less stable than the "non-condensed" multiple-ring type in which no carbon atoms are thus shared, the latter type is to be preferred. Poly-nuclear aromatic compounds (that is, those con-

taining more than one ring) of the non-condensed type are thus the more desirable of such aromatic compounds.

Preferred combinations to make up my new solvent include:

About 25% to 75% of o-dichlor benzene, ethyl dichlor benzenes, or ethyl chlor benzenes with one or more of the following:

Hexachlor diphenyl oxide  
Trichlor diphenyl oxide  
Monochlor benzophenone  
Benzophenone  
Phenyl acetate  
Phenol  
O-phenyl phenol  
Dibutyl phthalate  
Dichlorcyclohexanol  
Methyl salicylate  
Lauryl alcohol  
Tri-ethanol amine

The chlorinated diphenyl oxide compounds referred to above are compounds containing an average number of chlorine atoms equivalent to that indicated.

Of the specific compounds mentioned in this application all are more or less effective carbon binder solvents when used individually, although the highest efficiency is obtained with combinations as explained above. The individual examples of the immediately preceding list are among the best of the compounds which may be utilized by themselves.

Chlorine, bromine, and fluorine are the halogens most desirable in both the oxygen-free and oxygen-containing compounds, fluorine forming particularly stable compounds which are no longer so difficult to prepare as formerly. Methods of preparing fluorine compounds which will be found satisfactory for use in my solvent are described, for instance, in U. S. Patent No. 2,013,000, Example IV, and in U. S. Patent No. 2,013,050, Example X. My invention, of course, is not to be considered as involving any particular method of preparation of the components nor is it intended to be limited by any such method or methods. Iodine is quite expensive and the supply limited. Chlorine is the least expensive and most commercially available of all the halogens, and bromine is of especial value when the compounds are used in conjunction with lead anti-knock compounds. Iodine, and to some extent bromine, are also themselves effective as constituents in anti-knock compounds.

As the exact manner in which my solvent constituents act upon the carbon deposit is not entirely understood, I do not intend my invention to be restricted by any explanation or theory. However, the two types of solvents mutually aid one another in attacking the gummy carbon binders, for it has been found that the effectiveness of their joint action is more than the cumulative effect of the two when used separately.

The substitution of halogen in an organic compound lowers the volatility without of necessity causing solidification and thus enables the use of a number of the most effective types of solvents which would otherwise be too highly volatile at engine temperatures. The presence of the halogen in certain instances enhances the solvent action of the compounds and, therefore, makes available more effective compounds. It also reduces the inflammability of the composition. It has been observed that the degree of halogena-

tion modifies the effectiveness of the composition. The halogen also aids in the removal of metal residues of anti-knock constituents, and in some cases, has other desirable effects.

- 5 The action of my new solvent composition may sometimes be improved by the use of a more or less complex mixture of one or both of the two components used. This complexity may result from (a) the production of a plurality of compounds obtained by the halogenation process, as, for example, the chlorination of diphenyl which is capable of producing a large number of chlorine-bearing compounds differing as to the number and location of the chlorine atoms in the molecule; or (b) the use of a product resulting from the halogenation of a complex organic material such as certain still fractions and solvent-extraction fractions obtained in the separations of petroleum products and coal-tar products.
- 10 It is of advantage to use a combination of materials which will have a fairly wide range of volatility, in order to have an appreciable proportion of the solvent present in both the liquid and vapor phases over a wide range of temperatures. This condition promotes the carrying of the solvent to all parts of the combustion chamber and the condensation of a sufficient amount where needed. It is additionally advantageous to use at least one component which has an extremely low vapor pressure at room temperature, preferably less than atmospheric pressure at a temperature of about 250° C. A mixture of the products obtained by chlorinating benzene until it contains an average of about two atoms of chlorine per molecule with the product obtained by chlorinating diphenyl ether until the average chlorine content is about six atoms per molecule is very effective in this manner.
- 15 The more volatile portions of my solvent aid in carrying the less volatile portions to all parts of the combustion chamber and also condense during the compression stroke on the walls of the cylinder, cylinder head, piston head, valves, valve stems, etc. After the fuel has been exploded, there remains sufficient solvent to act effectively upon any carbon binder already deposited and inhibit the deposition of any more.
- 20 The relative proportions of halogenated oxygen-free organic constituents and oxygen-bearing organic constituents in the new solvent comprising my invention may vary within wide limits, depending upon the particular materials used, the kind of fuel to which the solvent is to be added, and the kind of engine employing the fuel, a very minor proportion of the more active components at times being quite effective. The ratio of the amount of halogenated oxygen-free organic constituents to the amount of oxygen-bearing organic material usually may vary from about one to ten, up to about ten to one, but preferably only from about one to two, up to two to one. For most applications a solvent comprising substantially equal amounts of each type has been found very satisfactory.
- 25 The amount of the solvent combination to be added to the fuel will depend upon the type of fuel and the type of engine using the fuel, and may vary over wide limits, for example, generally from about .001% to about .1% by weight based on the fuel. The amount will also depend upon the composition of the solvent and, for certain solvent compositions, less than .001% may be an effective amount. The upper limit of the amount which may advantageously be
- 30
- 35
- 40
- 45
- 50
- 55
- 60
- 65
- 70
- 75

mixed in the fuel is usually controlled by the effect of the added solvent on the carburetion of the fuel. When the solvent is largely composed of high boiling (i. e., non-volatile) materials too large an amount will interfere with proper carburetion. When the solvent is principally composed of materials in the lower range of boiling points, e. g. 140° C. (i. e. of relatively higher volatility), much larger amounts are permissible, for example up to about 0.5%. In the average gasoline for use in the ignition type four-stroke gas engine, such as is usually employed in automobiles, the solvent should be present in the gasoline in an amount of from about .005% to about .05%. A preferred amount for such conditions is about .01%.

For use in heavier fuels and especially those employed in automotive and stationary Diesel engines, a larger amount is usually desirable, say from about .01% to about .1% and preferably about .02%.

For use in two-stroke engines and in air-cooled engines of all types, the optimum amount of solvent in the fuel is about the same as that for Diesel engines, and in certain applications may be considerably higher.

Proper stability of the components of the solvent combination is an important factor. Since the materials are to be exposed to relatively high surface temperatures in the combustion chamber, they should be particularly resistant to thermal decomposition and also, since it is an advantage for at least part of the solvent to exist in the vapor phase in the combustion chamber to facilitate proper distribution, the materials chosen should preferably be capable of distillation at atmospheric pressure without appreciable decomposition.

Resistance to hydrolysis, although not essential, is a preferred characteristic, because of the tendency of moisture to condense on the walls of the cylinders, pistons, etc. when the engine is operated at low temperatures or for short intervals. Under these conditions, easily hydrolyzed halogen compounds will tend to produce hydrogen halides which will cause corrosion of the internal parts of the engine and therefore the least corrosive compounds are generally desired for use in most types of engines.

The superiority of my engine fuel has been demonstrated commercially by its highly successful use in automobile, truck and bus engines. In these cases, the solvent is mixed with the usual gasoline or heavier fuel before use, or may be directly injected into the combustion chamber, or may be added by any other practicable means. More detailed methods are given below. An important application of my invention is to Diesel engines where previously considerable difficulty has been met with in the form of carbon deposits which have militated against the more widespread use of this type of engine. The solvent constituents may be added by any practicable means to the ordinary Diesel engine fuel, much as in the case of spark-ignition-type engines. Many other specific applications of this invention have been made and will occur to those acquainted with the art, and this invention is intended to include all such applications.

While it is contemplated that the solvent will be introduced into the engine by dissolving in, or mixing with the fuel, it may also be introduced into the engine in other ways, either undiluted, or diluted, or in the form of a sus-

pension or emulsion in water. For example, either of the following means may be employed:

1. The solvent, preferably in the form of a vapor, mist, or spray, along with a small stream of air, is introduced into the combustion chamber, usually by admitting into the intake manifold.
2. The solvent is introduced, either directly into the combustion chamber or into the intake manifold, by means of some form of injector, usually mechanically actuated and preferably such as to produce a fine mist or spray.

15 The engine fuel according to my invention will then contain my new solvent comprising the combination of at least one representative of each of the types of compounds disclosed to inhibit the formation and aid in the removal of carbon deposits. It is usually preferable, but not absolutely necessary, that at least one of the solvents be of the aromatic series. The two components described have a cooperative dissolving effect, each enabling the other to work more quickly and completely.

As the prior art, notably Midgley, would indicate, such a fuel is ideal when used in conjunction with an anti-knock compound such as tetra-ethyl lead since the organic halogen compounds 30 are effective in promoting the conversion of the lead in the lead oxide formed as a result of combustion into a lead halide which will be volatile and therefore readily removed by the exhaust gases. Certain combinations of the materials 35 contemplated also have the effect of inhibiting the deleterious effects of lead deposits.

Fuel containing iron or nickel carbonyl as an anti-detonating agent will also be greatly improved when compositions of the type described 40 are added thereto.

As previously indicated, it is among the objects of this invention to provide a metal-containing anti-knock internal combustion engine fuel having my solvent added thereto which will have the 45 additional effect of converting the metal oxide formed into an easily removable product, and yet not causing appreciable corrosion.

As specific examples of combinations of compounds which are within the scope of this invention and are desirable in use with anti-knock compounds such as tetra-ethyl lead are:

- I. The combination of one or more brominated aliphatic hydrocarbons such as butylene dibromide, and amylen dibromide with:
    - (a) Unhalogenated oxygen-bearing aromatic compounds such as diphenyl ether, benzophenone.
    - (b) Brominated oxygen-bearing aromatic compounds, e. g. brominated diphenyl ether.
    - (c) Chlorinated oxygen-bearing aromatic compounds, e. g. chlorinated diphenyl ether.
  - II. The combination of one or more brominated aromatic hydrocarbons such as brominated benzene, brominated diphenyl, brominated naphthalene, brominated toluene, brominated ethyl benzene, with (a), (b), or (c) above.
- For satisfactory results an excess of halogen must be present in order that the lead or other metal may be completely combined and effectively removed. If this excess is present in the form of an easily hydrolyzed aliphatic compound, the unutilized portion may hydrolyze to some extent

causing appreciable corrosion. On the other hand, if no more than the amount of halogen needed to combine with the lead be present in the aliphatic compound and the excess halogen be present in an aromatic compound, then the unutilized excess will not hydrolyze and cause corrosion. If such carbon binder solvents as I have indicated above for use in metal containing engine fuels are utilized and the excess of halogen is present in an aromatic compound, then the effect of this form of my new solvent will be both to inhibit carbon formation and also to aid in the removal of the metal in a most efficient manner without causing corrosion. The advantages of such a combined operative effect are obvious.

As previously indicated, my new solvent which I have broadly described is also suitable for use by itself and need not necessarily be added to a fuel. It may, for instance, be injected into an engine which is not running but preferably still hot. Then on starting it after a period of time, the released carbon will be removed by the exhaust gases. Other occasions for its use are apparent to those concerned with the removal of similar organic deposits.

Other modes of applying the principle of my invention may be employed instead of the one explained, change being made as regards the ma-

terials employed in carrying out the process, provided the ingredient or ingredients stated in any of the following claims or the equivalent of such stated ingredient or ingredients be employed.

5 I, therefore, particularly point out and distinctly claim as my invention:

1. As a composition of matter a normally liquid organic solvent comprising (a) a halogenated aromatic monocyclic hydrocarbon and (b) a halogenated aromatic ether, said compounds having a vapor pressure below atmospheric at 170° C.

10 and being sufficiently stable so as not to substantially decompose either when boiled at atmospheric pressure or under the conditions encountered in the combustion chamber of an internal combustion engine.

15 2. A composition in accordance with claim 1 in which (a) is halogenated benzene.

20 3. A composition in accordance with claim 1 in which (a) is dichlor benzene.

25 4. A composition in accordance with claim 1 in which (b) is halogenated diphenyl ether.

5. A composition in accordance with claim 1 in which (a) is ortho-dichlor benzene and (b) is hexa-chlor diphenyl ether.

6. A composition in accordance with claim 1 in which at least one of the named halogenated organic compounds is alkylated.

CARL F. PRUTTON.